

## UNITED STATES PATENT OFFICE

CHARLES T. HENNIG, OF BARBERTON, OHIO

## METHOD OF PURIFYING FERROUS METALS

No Drawing.

Application filed August 22, 1928. Serial No. 301,434.

This invention relates to the manufacture of steel and especially to steel manufactured by the basic open hearth process. Heretofore sulphur has been considered to be a very objectionable constituent in steel and it has been the practice in steel plants to go to great trouble and expense to hold the sulphur content of the steel within a very narrow range of limits. It has been very difficult to remove sulphur from the metal, in the open hearth process, because the elimination of sulphur requires high heat and a reducing condition whereas an oxidizing condition obtains in the basic open hearth furnace. In practicing the basic open hearth process the principal elements that are eliminated from the metal are silicon, manganese, carbon, phosphorus and some sulphur. The most important of these are phosphorus and carbon and since phosphorus requires an oxidizing condition in the furnace, a condition which would eliminate sulphur would drive the phosphorus back from the slag into the metal. Because of the difficulty of eliminating sulphur, by the basic open hearth process, it has been customary for the steel plants to avoid a high sulphur content in the finished steel by using metals, in the charges, that did not contain an excessive amount of sulphur. Heretofore, when the steel has been high in sulphur, it has caused much difficulty in the rolling mills because of the tendency of the ingots and billets to crack and it is one of the objects of the present invention to overcome this difficulty in steels containing, what would ordinarily be considered, an excessive amount of sulphur. My invention, therefore, enables the use of metals, in the basic open hearth furnace, that have a higher sulphur content than would heretofore have been considered good practice and as such metals have a lower market value than low sulphur metals, my invention effects material economies in the manufacture of the steel.

The development of the automobile industry has resulted in a large demand for deep-drawing steels and it is one of the objects of the invention to produce deep-drawing steels of a superior quality. It is a fur-

ther object of the invention to produce steel that will have an exceptionally good surface and also be uniform and without hard spots. I have found that hard spots in steel are usually manganese and iron silicates and oxides and the elimination of these segregations of manganese and iron silicates and oxides results in steel which has clean surfaces and is more ductile and better adapted for deep-drawing and for the manufacture of wire. The steel also has better physical properties. The elimination of these segregations from steel that is to be used in making wire is especially desirable because hard spots in the wire cause lack of uniformity in drawing and the hard spots tend to tear the dies, thereby forming nicks in the wire which reduce the strength of the wire and are points at which the wire will break when bent.

In deep-drawing steels these hard spots also result in tearing of the metal and difficulty in shaping the metal in the dies.

In steel that is to be coated with zinc, lead, tin, nickel or other metals it is very important to have clean and uniform surfaces because, when the metal is pickled for the purpose of taking off scale, the acid will penetrate into the steel, if the surfaces are defective, and collect around the inclusions with the result that when the sheets are later heated in the coating process the hydrogen that is liberated by the reaction of the acid on the steel is driven to the surface and raises the coating in the form of blisters, thereby producing a defective product.

My invention has for a further object the production of "rim" steel having a thicker and denser skin so that when this steel is rolled out into sheets it will have a clean and uniform surface. In the manufacture of "rim" steel the metal is usually very active when poured into the molds and by the use of my invention the activity of the metal, in the molds, is kept under better control and the ingots have clean and dense surfaces which are not so sensitive to heating and burning in the soaking pits and heating furnaces. This is very important because, with a less dense skin, blow-holes form close to the surface and the fire attacks the surface and

makes spots which develop into seams in rolling.

It is a further object of my invention to reduce the amount of deoxidizer, such as 5 aluminum, silicon or manganese, that is required in the manufacture of "killed" steel. The term "killed," as applied to steel, refers to a steel that has been practically degasified in the open hearth furnace but in pouring 10 such steel into the molds it is customary to add a deoxidizer for the purpose of eliminating some of the iron and manganese oxide that is still in the steel and, by the use of my invention, the metal is so completely 15 deoxidized, in the open hearth furnace, that very little, if any, deoxidizer is required in the molds.

In practicing my invention I utilize soda, in the form of commercial soda ash, as the 20 means for reducing the iron and manganese oxides and silicates and otherwise purifying the metal. In my Patent 1,717,153, June 11, 1929, I disclosed a method of desulphurizing and purifying steel by the use of soda 25 ash and while that method has been found to produce beneficial results it has not been entirely satisfactory because the soda has a tendency to be more or less erratic in its action and the results sought for could not 30 always be obtained with certainty. My present method is, therefore, an improvement on the method disclosed in my Patent 1,717,153 and this improvement eliminates all uncertainty as to the results and permits a sub- 35 stantially uniform practice in the steel plant with practically uniform results.

Steels produced by my improved method, whether "rim" or "killed" steels, are practically free from dissolved iron oxides and 40 the segregations of iron and manganese oxides and silicates that have given trouble heretofore in the manufacture of steel by the standard basic open hearth method. When steels made by my improved method are 45 rolled out into thin sheets these sheets have a smooth, clean surface with a high lustre. Such sheets are especially well adapted for being coated with tin, lead, zinc or nickel and because of the character of the surfaces 50 the coating is uniform and so firmly united with the surface of the sheet that a thinner coating may be used, thereby a saving in the cost of coating is made possible.

In practicing my invention, in the basic 55 open hearth process, I introduce into the molten metal, and preferably into the molten iron before it is poured into the open hearth furnace, a purifying material which consists essentially of a mixture of soda ash and a 60 controlling substance therefor, such as manganese dioxide, which will insure reliable results. The purifier may vary as to its composition but in addition to the materials specified, contains some lime to raise the melting 65 point of the soda ash, and I have found

that the following composition is entirely satisfactory:

|                                                        |            |
|--------------------------------------------------------|------------|
| Commercial soda ash (NA <sub>2</sub> CO <sub>3</sub> ) | 90%        |
| Calcium oxide (CaO), as limestone                      | 3 to 4%    |
| Manganese dioxide (MnO <sub>2</sub> )                  | 1/4 to 1%  |
| Chlorine, as calcium chloride (CaCL <sub>2</sub> )     | about 1/2% |

and the balance impurities in the form of 75 silica, magnesia, iron and aluminum. The materials, in the proportions specified, may be melted at a temperature of from 2300 to 2600° F. and then run out onto iron plates 80 and broken up into pieces of from 1/2 inch to 3 or 4 inches in size. From 2 to 4 pounds of the purifier, per ton of iron, treated, will give satisfactory results. The purifier may be put into the transfer ladle, either before 85 or during the pouring of the metal thereinto from the mixer or the blast furnace ladle, and the action of the purifier is very pronounced. The soda ash is broken up and the carbon dioxide and other gases that are released produce a violent boiling of the 90 metal and this causes the purifier to be diffused throughout the body of the metal. The soda ash takes the oxygen from the dissolved iron oxides and the manganese oxide 95 and also reacts with the iron and manganese silicates forming sodium silicate and metallic iron and manganese. The sodium silicate rises to the surface of the metal and enters the slag and tends to make the slag more liquid. 100

Instead of melting the materials forming the purifier they may be mixed dry, in a pulverized form, and a suitable binder added and then formed into briquets. Instead of using a binder water may be added which 105 will, through its action on the soda, produce heat and harden the materials when they are pressed into briquets.

When the purifier is introduced into the open hearth furnace it enters the slag and 110 makes it more liquid. This facilitates the boiling of the metal and causes it to be forced up through the slag, in the form of spouts or guys, and as the metal passes through the slag it is washed by it and when above the 115 slag the furnace gases are permitted to oxidize the impurities. The soda alone has a lower specific gravity than the usual open hearth furnace slag but the manganese oxide, which is present in the purifier, increases the 120 gravity so that the lumps or briquets of the purifier will sink through the slag and float on the metal where they will melt and the purifier will have an opportunity to react with the impurities in the metal. 125

Having thus described my invention, I claim:

1. The herein-described method of purifying steel in the course of its manufacture by the basic open-hearth process which consists 130

in introducing into the molten metal a de-  
oxidizing material in the form of an intimate  
mixture comprising commercial soda ash and  
manganese dioxide and wherein the soda ash  
5 is over three-fourths of the mixture and  
the manganese dioxide is an effective amount,  
up to five per cent, for controlling the action  
of the soda ash as and for the purpose de-  
scribed.

10 2. The herein-described method of purify-  
ing steel in the course of its manufacture by  
the basic open-hearth process which consists  
in introducing into the molten metal a de-  
oxidizing material in the form of an inti-  
15 mate mixture comprising commercial soda  
ash, a calcium compound and manganese di-  
oxide and wherein the soda ash is over three-  
fourths of the mixture, the calcium compound  
has a calcium oxide content that is an effective  
20 amount, up to ten per cent, to substantially  
raise the melting point of the soda ash, and  
the manganese dioxide is an effective amount,  
up to five per cent, for controlling the action  
of the soda ash as and for the purpose de-  
25 scribed.

3. The herein-described method of purify-  
ing steel in the course of its manufacture by  
the basic open-hearth process which consists  
in introducing into the molten metal lumps  
30 of a deoxidizing material in the form of an  
intimate mixture comprising commercial  
soda ash, a calcium compound and manganese  
dioxide and wherein the soda ash is over  
three-fourths of the mixture, the calcium  
35 compound has a calcium oxide content that is  
an effective amount, up to ten per cent, to  
substantially raise the melting point of the  
soda ash, and the manganese dioxide is an  
effective amount, up to five per cent, for con-  
40 trolling the action of the soda ash as and  
for the purpose described.

In testimony whereof, I hereunto affix my  
signature.

CHARLES T. HENNIG.

45

50

55

60

65